

## UNITED STATES PATENT OFFICE

2,054,775

## DEWAXING HYDROCARBON OIL

Ernest Frank Pevere, Beacon, N. Y., assignor to  
The Texas Company, New York, N. Y., a corporation of Delaware

No Drawing. Application May 7, 1935,  
Serial No. 20,190

5 Claims. (Cl. 196—19)

This invention relates to dewaxing hydrocarbon oil and more particularly to the removal of wax from mineral lubricating oil stock for the production of low pour test lubricating oils.

5 The invention contemplates a solvent dewaxing process wherein a solvent selected from the dialkyl ethers of methylene, such as methylene dimethyl ether or methylal is employed. Methylal, for example, has the chemical formula 10  $\text{CH}_2(\text{OCH}_3)_2$  and may be prepared by reacting formaldehyde with methyl alcohol.

Instead of the dimethyl ether, methylal, it is contemplated that the diethyl and dipropyl ethers of methylene may also be employed, including 15 both the iso and the normal forms of the dipropyl ether.

More specifically, the invention comprises mixing a wax-bearing mineral oil fraction with a solvent comprising methylal in proportions such 20 that at temperatures of 0° F. and below the solvent has substantially complete solvent action on the liquid constituents of the oil and substantially no solvent action upon the solid waxy constituents of the oil. This mixture is chilled to temperatures of the order of 0° F. and below, depending 25 upon the desired pour test of the dewaxed oil, to precipitate the wax constituents. The precipitated wax constituents are then separated from the cold mixture by mechanical means such as filtration, centrifuging or settling.

30 I have discovered that methylal possesses properties which render it suitable as a dewaxing solvent. This solvent has anti-solvent properties for paraffin wax and in addition possesses comparatively high solvent power for mineral oil so that it may be employed alone as a satisfactory dewaxing solvent liquid. Its selective solvent action as between solid and liquid hydrocarbon constituents of wax-bearing mineral oil, at temperatures of around 0° F., is such that when dewaxing 35 with this solvent liquid the pour temperature of the dewaxed oil will correspond to the dewaxing temperature and in some cases will have a pour temperature below the dewaxing temperature.

40 In some cases, as for example in the case of heavy viscous oils, such as residual cylinder stocks, it may be desirable to employ a diluent solvent in conjunction with the methylal. Accordingly in 45 dewaxing such stocks, the wax-bearing oil may be mixed with a solvent mixture composed of methylal and solvent liquids of the character of benzol and its homologs or a light petroleum fraction, such as naphtha, or a petroleum fraction comprising mainly the normally gaseous hydrocarbons, such as propane and butane.

In order to more fully describe the invention, reference will now be made to the following example in which a wax-bearing distillate derived from Mid-Continent crude was dewaxed with methylal. The tests on the wax-bearing distillate 5 were substantially as follows:

|                                   |            |
|-----------------------------------|------------|
| Gravity A. P. I.                  | 22.9       |
| Saybolt Universal vis. at 210° F. | 73 seconds |
| Pour test                         | 105° F.    |

10

One volume of the foregoing oil was mixed with three volumes of methylal. The resulting mixture was chilled to 6° F. to precipitate the wax constituents and while maintained at this temperature the cold mixture was filtered to separate 15 the precipitated wax constituents.

The solvent was removed from the resulting filtrate by distillation and the remaining dewaxed oil amounting to about 70% of the original wax-bearing distillate, had a pour test of 20 —5° F. with a solid point at —8° F.

It will be observed that in the foregoing example the dewaxed oil had a pour test temperature of 11° below the dewaxing temperature.

The proportion of methylal to oil undergoing 25 dewaxing may vary considerably from that specified in the foregoing example. Thus it is contemplated that the proportion of methylal to oil may be either less or greater than that mentioned, as for example, from 2 to 4 volumes of 30 methylal to one volume of wax-bearing oil.

In the case of heavy viscous oils where it is desired to use a modifying or diluent solvent as already indicated, the proportion of methylal to diluent solvent will depend to some extent upon 35 the character of the oil undergoing treatment and also upon the nature of the diluent being used. In the case of reduced residual cylinder stocks, for example, the proportion of methylal to diluent liquid may comprise around one part 40 of methylal to 2 or 3 parts of diluent solvent.

The solvent of my invention is adapted to the separation of wax from petroleum oil or from either residual or distillate fractions thereof. It is also adapted to the treatment of wax 45 concentrates for the purpose of effecting the separation between the wax and oil constituents.

Obviously many modifications and variations of the invention, as hereinbefore set forth, may be made without departing from the spirit and 50 scope thereof, and therefore only such limitations should be imposed as are indicated in the appended claims.

I claim:

1. In the dewaxing of wax-bearing mineral 55

oil, the method which comprises mixing the oil with a solvent comprising methylal, chilling the mixture to precipitate the wax constituents, and separating the precipitated wax constituents 5 from the cold mixture.

2. In the dewaxing of wax-bearing mineral oil, the method which comprises mixing the oil with methylal, chilling the mixture to precipitate the wax constituents, and separating the pre- 10 cipitated wax constituents from the cold mixture.

3. In the dewaxing of wax-bearing mineral oil, the method which comprises mixing the oil with methylal in the proportion of about one volume 15 of oil and from two to four parts of methylal, chilling the mixture to a temperature of the order of 0° F. and below to precipitate the wax constituents, and removing the precipitated wax constituents from the cold mixture.

20 4. In the dewaxing of heavy viscous wax-bearing mineral oil the method which comprises mixing the oil with a solvent composed of methylal and a diluent solvent of the character of benzol

in proportions such that at temperatures of 0° F. and below the mixture has substantially complete solvent action on the liquid constituents of the oil, and substantially no solvent action on the solid waxy constituents of the oil, chilling 5 the mixture to temperatures of 0° F. and below to precipitate the wax constituents and removing the wax constituents thus precipitated from the cold mixture.

5. In the dewaxing of wax-bearing mineral oil, 10 the method which comprises mixing the oil with a solvent liquid comprising a dialkyl ether having the formula:



where R—R represent alkyl radicals selected from the group consisting of methyl, ethyl and 20 propyl, chilling the mixture to precipitate the wax constituents, and separating the precipitated wax constituents from the cold mixture.

ERNEST FRANK PEVERE.